

March 8, 1960

F. PAWLEK

2,927,898

PERMANENT MAGNET MATERIAL

Filed March 30, 1959

*Triangular Plot of the  
Three-Component System of*

$Fe_2O_3-PbO-SiO_2$   
in mol percent



*Inventor:*

Franz Pawlek  
By *Eni D. Meek*  
Patent Agent

# United States Patent Office

2,927,898

Patented Mar. 8, 1960

1

2,927,898

## PERMANENT MAGNET MATERIAL

Franz Pawlek, Berlin-Lichterfelde-West, Germany, assignor to Licentia Patent-Verwaltungs-G.m.b.H., Hamburg, Germany

Application March 30, 1959, Serial No. 802,814

7 Claims. (Cl. 252—62.5)

The present invention relates to materials for permanent magnets and to a method for making such materials; more specifically, this invention pertains to a magnetic material composed of a mixture of various metallic oxides, and to the manufacture of such mixture. The present application is a continuation-in-part of my copending application Serial No. 456,070, filed on September 14, 1954, now abandoned, for Permanent Magnet Material.

It is well recognized that a satisfactory material for permanent magnets must possess high remanence and should also have a high coercive force. At the same time, economic considerations demand that the material be composed of constituents which are not so expensive as to make their use prohibitive. Furthermore, it is desirable that permanent magnet materials be composed of constituents which are readily available.

There are certain magnetic materials on the market, such as alloys, which have reasonably good magnetic properties in terms of remanence and coercive force. However, many of these materials include such metals as cobalt and nickel which are difficult to extract from their ores and which, in times of emergency, are considered strategic materials to be reserved primarily for strategic goods.

On the other hand, there are magnetic materials, such as iron, which are readily available at comparatively reasonable prices, but which do not possess the above-mentioned magnetic characteristics to the desired degree.

Therefore, any material which is characterized, at the same time, by ready availability, low cost, and favorable magnetic properties constitutes a very valuable addition to the present store of engineering achievements.

Accordingly, it is an object of the present invention to provide a permanently magnetic material which is characterized by high values of remanence and coercive force and which, at the same time, is composed of inexpensive and readily available constituents.

It is another object of the invention to provide a reasonably simple and convenient method of producing the material mentioned above.

It is a further object of this invention to heat a mixture of  $Fe_2O_3$ ,  $PbO$ , and  $SiO_2$ , said mixture forming a three component system the proportions of which are represented in mol percent in an equilateral triangle, whereby the composition of the mixture is defined by a pentagon inside said triangle, said pentagon having the following corners or coordinates in mol percents:

|                   |               |                |
|-------------------|---------------|----------------|
| 65 of $Fe_2O_3$   | 30 of $PbO$   | 5 of $SiO_2$   |
| 75 of $Fe_2O_3$   | 20 of $PbO$   | 5 of $SiO_2$   |
| 81 of $Fe_2O_3$   | 15 of $PbO$   | 4 of $SiO_2$   |
| 84.5 of $Fe_2O_3$ | 15 of $PbO$   | 0.5 of $SiO_2$ |
| 76 of $Fe_2O_3$   | 23.5 of $PbO$ | 0.5 of $SiO_2$ |

The above mixtures are heated, i. e., fired in an air current at a sintering temperature between 700° C. and 1,200° C. for a period of time between three and four hours.

2

Other and further objects and advantageous features of the present invention will hereinafter more fully appear in connection with the drawing which constitutes a triangular plot, in mol percents, of the three-component system of  $Fe_2O_3$ ,  $PbO$  and  $SiO_2$ .

As mentioned in the foregoing, the permanently magnetic material according to the present invention can be prepared very inexpensively. The inexpensive nature of the material is attributable to the easy availability of its constituents and to the simplicity of the method of manufacturing the material, as will be explained in the following:

An aqueous slurry should first be prepared by (1) pulverizing metallic oxides of the type and in the proportions falling within the pentagon defined in the foregoing, and (2) mixing the resulting powder with water.

The water is then filtered off, and the remaining solid dried by applying moderate heat. In order to facilitate the subsequent molding steps and the removal of the magnetic material from the molds, a small amount of paraffin, dissolved in trichloroethylene, may at this time be added to the mixture to act as a lubricant. Alternatively, stearic acid of other suitable waxes may be employed for the same purpose.

Following the addition of the lubricant, the mixture will be dried again, permitting the solvent of the lubricant to evaporate. The powdered mixture should then be pressed into molds of any desired shape, whereupon the pressed material will be fired in an air current for a period of between three and four hours at a temperature between 700° and 1,200° C. Finally, the pressed material is cooled and removed from the molds.

While it will be understood that the magnetic characteristics of the finished magnetic material depend somewhat upon the percentage of the various constituents used in formulating the material, I have found that suitable mixture ratios are the following:

|                | $Fe_2O_3$ | $PbO$ | $SiO_2$ | Remanence in Gauss | Coercive Force in Oersted |
|----------------|-----------|-------|---------|--------------------|---------------------------|
| 1. Mol percent | 65        | 30    | 5       | 1,380              | 1,650                     |
| 2. Mol percent | 75        | 20    | 5       | 1,410              | 3,200                     |
| 3. Mol percent | 81        | 15    | 4       | 1,000              | 3,500                     |
| 4. Mol percent | 84.5      | 15    | 0.5     | 1,300              | 2,100                     |
| 5. Mol percent | 74        | 25    | 1       | 1,400              | 1,900                     |
| 6. Mol percent | 72.45     | 23.85 | 3.7     | 1,700              | 1,850                     |
| 7. Mol percent | 77        | 20    | 3       | 1,800              | 2,250                     |
| 8. Mol percent | 78.63     | 19.15 | 2.22    | 2,000              | 2,100                     |
| 9. Mol percent | 81.65     | 16.4  | 1.95    | 1,600              | 2,800                     |

Referring to the drawing it will be evident that the first four examples represent the coordinates at four corners of the pentagon indicated by the reference numerals 1 to 4, respectively; the last five examples lie within the pentagon. The best results are obtained with the composition of Example 8.

Regardless of remanence, the following compositions render high coercive forces:

65-80 mol percent of  $Fe_2O_3$   
20-30 mol percent of  $PbO$   
1-5 mol percent of  $SiO_2$

These mixtures are to be fired preferably for four hours at a sintering temperature of 1,000° C. in a current of air and should be cooled thereafter.

The resistivity of the magnetic materials thus formed was found to be in the range of  $10^{10}$  ohm-cm.

It will be noted that the above-described characteristics show a significant improvement over the known types of permanently magnetic materials. In addition, the new method of making the material is simple and depends only upon inexpensive and easily available constituents,

Furthermore, the property known as the B-H factor (the product obtained by multiplying the magnetizing field strength by the resulting magnetic-flux density) is extremely high for the new material. The B-H product or factor for a given material often is of value as a criterion for use in selecting a permanently magnetic material.

While I have described my invention in connection with specific compositions and examples of the new method, I wish it to be understood that other and further modifications, apart from those shown or suggested herein, may be employed without departing from the spirit and scope of my invention, which may be defined by the appended claims.

What is claimed is:

1. A permanently magnetic material prepared by heating a mixture of  $Fe_2O_3$ ,  $PbO$ , and  $SiO_2$ , to a temperature between 700° and 1,200° C., said mixture falling within the bounds of a pentagon defined on an equilateral triangular plot of the three components of the mixture, each side of the triangular plot representing one of the components in mol percent from 0 to 100%, the pentagon being represented by the following coordinates:

| $Fe_2O_3$ | $PbO$ | $SiO_2$ |
|-----------|-------|---------|
| 65        | 30    | 5       |
| 75        | 20    | 5       |
| 81        | 15    | 4       |
| 84.5      | 15    | 0.5     |
| 76        | 23.5  | 0.5     |

2. A permanently magnetic material prepared by heating a mixture of 65 to 80 mol percent of  $Fe_2O_3$ , 20 to 30 mol percent of  $PbO$ , and approximately 1 to 5 mol percent of  $SiO_2$  to a temperature between 700° to 1,200° C.

3. A method of producing a permanently magnetic material comprising the steps of preparing a mixture in the three-component systems  $Fe_2O_3$ — $PbO$ — $SiO_2$  defined with in a pentagon having as corners on an equilateral triangular plot the following coordinate mol percentages:

| $Fe_2O_3$ | $PbO$ | $SiO_2$ |
|-----------|-------|---------|
| 65        | 30    | 5       |
| 75        | 20    | 5       |
| 81        | 15    | 4       |
| 84.5      | 15    | 0.5     |
| 76        | 23.5  | 0.5     |

and of heating said mixture between 700° and 1,200° C and cooling the product thus obtained.

4. A method according to claim 3, characterized in that the mixing ingredients are pulverized and converted into an aqueous suspension and that the heating is carried out in air current for three to four hours.

5. A method for producing a permanently magnetic material comprising the steps of mixing

65 to 80 mol percent of  $Fe_2O_3$

20 to 30 mol percent of  $PbO$

1 to 5 mol percent of  $SiO_2$

approximately

of heating said mixture between 700° and 1,200° C., and cooling the product thus obtained.

6. A permanently magnetic material prepared by heating a mixture of 78.63 mol percent of  $Fe_2O_3$ , 19.15 mol percent of  $PbO$  and 2.22 mol percent of  $SiO_2$  to a temperature between 700° and 1,200° C.

7. A permanently magnetic material prepared by heating a mixture of approximately 74 mol percent of  $Fe_2O_3$ , approximately 25 mol percent of  $PbO$ , and approximately one mol percent of  $SiO_2$  to a temperature between 700° and 1200° C.

References Cited in the file of this patent.

UNITED STATES PATENTS

1,821,208 Dahlberg \_\_\_\_\_ Sept. 1, 1931  
2,762,777 Went et al. \_\_\_\_\_ Sept. 11, 1956

FOREIGN PATENTS

697,219 Great Britain \_\_\_\_\_ Sept. 16, 1953

OTHER REFERENCES

Harvey et al.: RCA Review, September 1950, page 346.  
Went et al.: Physical Review, vol. 86, pages 424-425  
(1952).

25

30

45

50